

Sept. 1, 1942.

H. COOPER

2,294,654

LEATHER COMPOSITE HAT BAND

Filed Sept. 13, 1938



Fig. 1



Fig. 2



Fig. 3



Fig. 4



Fig. 5

INVENTOR.

Himen Cooper

BY

Ostrolenk, Green & Maser

ATTORNEYS

## UNITED STATES PATENT OFFICE

2,294,654

## LEATHER COMPOSITE HATBAND

Himen Cooper, West Philadelphia, Pa.

Application September 13, 1938, Serial No. 229,655

1 Claim. (Cl. 2-181)

My invention relates to novel leather composites and the methods of making the same and more particularly it relates to a novel composite leather hat band and the process for making the same.

This application is a continuation in part of my co-pending application for patent No. 72,123 filed April 1, 1936, which matured into Patent No. 2,132,399.

It has long been customary to employ around the inside circumference of hats, a leather band commonly termed a sweat band. The hat band is made of leather because it must be air pervious and absorbent. This leather band which I term a hat band has the function of preventing the passage of perspiration of the head through to the felt of the hat. In addition, it contacts the head and positions the hat upon the wearer's head. The hat band further acts as a guard to prevent shape distortion of the hat.

A further important function of the hat band is to maintain proper fitting of the hat upon the wearer's head during the life of the hat. It has been found, however, that the ordinary leather hat band has a tendency to stretch under constant use causing the hat to loosen up after periods of wear.

I have discovered that a novel hat band may be formed from a composite of leather and fibrous material such as fabric which serves all the useful functions of the customary hat band and in addition has certain properties which render it superior to the leather hat band customarily used in this art.

A further important feature of my hat band lies in the fact that it can be made far less expensively than the leather hat band and is adapted to commercially compete with substitute hat bands of paper, pulp or fabric material which have hitherto been employed as cheap substitutes for the customary leather hat band. Such substitutes have been found to be unsatisfactory chiefly in wearing qualities and lack of strength.

I form my novel hat band from a composite of thin leather such as leather skiver or scrapings and a fibrous backing material such as fabric. Since it is imperative in all hat bands that a permeability to air be maintained, I have employed a novel method of joining the leather to the fabric.

I have discovered that by employing a cement that is free of fillers or foreign matter normally causing cement to become stiff or hardened when dry, i. e., by utilizing cement in a highly pure state, it remains soft after being dried, while at

the same time providing all of the necessary adhering properties. I have further discovered that by applying this cement in a fine spray so that it is atomized and uniformly distributed in an extremely thin film over the leather surface to be cemented with the fabric, so that the individual globules of the cement are prevented from coagulating with each other to form a hard stiff substance, the ultimate product retains the softness, "feel" and break of the original leather. The product of leather combined with fabric is stronger and "warmer" than leather alone. Thus, in practice, I spray in atomized form a latex cement free of fillers upon the leather so that the latex is deposited upon the leather in such fine individual globules that this cement does not seal or close up the pores of the leather. Similarly I may coat the fabric material with the cement and laminate the coated fabric to the coated leather by means of a light rolling pressure to secure a permanent bond therebetween. It is important to note that I employ a highly concentrated latex cement with no fillers inasmuch as such a cement affords a very soft and flexible bond between the leather and the fibrous material when the joining is effected as above set forth.

By properly stretching the leather in a single direction to a predetermined degree before combining it with the fibrous material with which it is joined, I can secure as a finished product a hat band with a predetermined degree of stretch. Since it is a desirable requisite of a hat band that it stretch, if it stretch at all, to a known degree this property of predetermined stretch of the composite is of special utility in a hat band.

As the layer of leather I may employ skivers of sheep skin, goat skin, cow-hide buffings. Similarly, skins of any animals customarily used as a source of leather may be employed. In addition to skivers, thicker or thinner leather sections may be employed. It is especially advantageous to use skivers as indicated because of their relative cheapness and because when composited in accordance with the method I have set forth they produce a hat band of the proper strength and the requisite qualities. In place of compositing fabric with the leather as I have indicated above I may employ paper or any other fibrous material. The particular materials employed are determined by the properties desired, and the wearing qualities necessary in the finished hat band.

It is an object of my invention to provide a novel hat band.

It is a further object of my invention to provide a novel hat band comprising a composite of leather and fabric joined in such a manner as to provide an air pervious composite.

It is a further object of my invention to provide a composite hat band comprising skivers and fabric joined by latex cement in such a manner as to provide an air pervious hat band.

It is a further object of my invention to provide a composite hat band of leather and fibrous material joined by a cement in such a manner as to provide an air pervious hat band.

These and further objects of my invention will become apparent from the more detailed description of my invention taken in connection with the drawing, in which:

Figure 1 is a perspective of the sweat band of my invention.

Figure 2 is a cross-section taken along the line 2—2 of Figure 1.

Figure 3 is a side elevation of a tank of treating liquor and a skin disposed therein.

Figure 4 is a plan view of the step of spraying the leather secured to a smooth surface in accordance with my invention.

Figure 5 is a side elevation of a composite of leather and stretchable knitted backing held in a curved position showing the give of the backing.

Referring now more specifically to the drawing, in Figure 1 is shown a hat band 1 comprising a layer of leather 2 secured to a backing 3.

In Figure 2 the composite is shown in detail and therein can be seen the leather 2 with the pores 4 secured to the backing 3 by the globules of cement 5. This figure illustrates the position of the globules of cement, such as latex, and the manner in which they are deposited onto the leather. By spraying this latex on to the leather, it assumes the form of globules, as seen, and tends to adhere to the solid portions of the leather without blocking the pores 4. Thus a good adhesion can be obtained while retaining air pervious qualities if such be desired and, at the same time, the adhesive, being in the form of soft and resilient globules, affords a soft feel to the composite.

Figures 3 and 4 illustrate the method which I employ to form my composite. In Figure 3 I show the leather or skiver 7 being treated in a tanning bath 8, contained in a tank 9, although, of course, this bath may be of fat liquor and the step represent any one of the final steps in the treatment of the leather. The factor of importance, of course, is that the leather be in a condition at least damp and preferably very moist or wet. While in the state of being damp and preferably wet, the leather 7 is smoothed out or "slickered on" to a smooth and rigid surface 10. This surface may, of course, be a Bakelite, glass, board, or linoleum covered board or any suitable smooth surface to which the leather will adhere in a wet condition. By suitably using a stick or a knife, the leather 7 is adhered closely to the smooth and rigid surface 10 and thereafter globules of a suitable flexible cement, as of latex, 11 are deposited onto the leather 7 by means of a spray 12. After the flexible cement 11 is deposited onto the leather 7, the backing 3 is applied thereto, preferably by means of a light rolling pressure such as applied by a rolling pin or the like. An effective bond is secured between the backing and the leather.

In Figure 5 is illustrated the composite of leather and fabric of my invention in which to avoid piping, I provide a backing 15 which pref-

erably is a knitted material, although it may be any suitable material that has a give or elasticity greater than the fleshy side 16 of the leather 17. In this figure, 18 represents the smooth side of the leather and 16 represents the fleshy side of the leather. In order that the surface 18 does not pipe or wrinkle when it is bent as shown in this figure, it is necessary that the backing 15 have a give or elasticity greater than the fleshy side of the leather 16 as shown. In that event, upon bending as shown here, the backing will not tend to constrict the leather but will give with the bend. Inasmuch as knitted fabric has the necessary give and, customarily, woven fabric does not, I prefer to use a knitted fabric. In the leather 17 are the pores 20 and it can be seen that in most cases the cement globules 21 position themselves on the solid portion of the leather and do not tend to block the pores.

I shall now describe the specific manner of making my composite. I first subject the skivers to a tanning operation to produce a soft and stretchy skiver. The tanning bath and the length of the tanning are carefully controlled to obtain the desired softness and stretch in the skiver as indicated.

After tanning, the skivers are dyed and placed upon wooden horses to drain. After the skivers have drained for a period of several hours and while still in the wet state, they are slickered onto a glass or any other suitable hard and smooth surface. Skivers are preferably twenty-four inches in width and they are pulled out to their full length so as to eliminate any wrinkles. If desired, pulling out can be effected so that the leather is stretched in this one direction so that it will have an ultimate predetermined stretch in a single direction only. Thus, in the finished product the exact stretch of the leather of the composite will be known. The fabric to which the leather is joined also controls the stretch.

The tanning operation which is a novel process that I have devised and produces new and unexpected results will be described in full hereinafter. This novel tanning process of my invention is of general application and produces a fine grain leather of excellent properties.

Skivers or skins spread out on the smooth glass surface are then dried. After this drying operation, the skivers or skins still adhere tightly to the glass and are somewhat damp. The fabric backing, viz. cloth, is then cut to the approximate length and width of the skiver. The cut fabric is then placed upon suitable frames and the skiver or leather skin and the fabric are sprayed with a latex compound. A suitable latex compound comprises:

|                                                     | Percent |
|-----------------------------------------------------|---------|
| Latex                                               | 68.0    |
| Water                                               | 16.5    |
| Casein                                              | 10.0    |
| Zinc                                                | 1.7     |
| Sulphur                                             | .8      |
| Ammonia                                             | .8      |
| Caustic potash                                      | .2      |
| Zinc salt of 2 mercaptobenzothiazole—10% of the wax | 1.4     |
| Mercaptobenzothiazole                               | .4      |
| Symmetrical dibeta-naphthyl para phenylene diamine  | .2      |

These proportions are according to weight. These ingredients and the proportions thereof may be varied. The ingredients are mixed at

room temperature to form a paste which is the cement. The cement is then passed through fine sieve to remove lumps.

It is to be noted that this cement composition is a highly concentrated latex containing curing agents. No fillers are used. In place of the latex composition above set forth other suitable cements may be employed such as a rubber cement containing a substantial quantity of oil and certain flexible millinery glues that contain castor oil. However, a latex compound capable of being sprayed to form individual globules is preferred since it has been found that the desirable properties of softness and flexibility plus weight are best secured with a latex cement.

This cement is sprayed onto the stretched leather through a fine nozzle. I have obtained satisfactory results with a  $\frac{1}{4}$  inch nozzle, and a pressure of 45 pounds per square inch. The cement is uniformly distributed on the surface of the leather in a very thin film. The globules of the cement are atomized so that they are substantially of the size of the grain of leather used. Thus, the globules of cement are deposited on the solid portions of the leather through natural adhesion and do not block up the pores or openings in the leather. In this way, by means of the sprayed latex a thin layer with very fine air holes is deposited on the leather. Thus a porous leather is joined to a porous fabric by means of an air pervious cement. In this way an air pervious composite is obtained.

Next the fabric is spread onto the sprayed leather to form a smooth layer thereon while the latex is still wet and while the leather is still held upon the smooth surface. The fabric and the leather are united by passing a light pressure thereover. This light pressure can be transmitted to the composite by means of a roll. The pressure upon the roll, however, must be carefully controlled so that the cement is not forced into the interstices which as above noted it is not desired to block.

Further the light pressure is believed to preserve the cement in more or less globule form so that the ultimate product has a very desirable soft feel. The combined leather and fabric are then left for about 24 hours on the glass until thoroughly dried. Because of the adherence of the leather to the glass above described no undesirable shrinkage takes place during the drying operation. When the cement dries, a firm unitary composite structure is had which is substantially unaffected by the presence of the cement which bonds the fabric to the leather. The cement remains soft and pliable; after drying the product may be used for wearing apparel and the like where porosity is necessary.

When the cement coats the fabric it lodges only onto the solid portions of the fabric and does not tend to block the openings in the fabric. Naturally the so coated fabric entirely retains its porous and air pervious properties.

This step of the application of the cement to the materials to be joined is of vital importance in my process since it is upon this step that the air perviousness of the finished composite depends. It is the fundamental principle of my invention that the cement should be applied to the fabric or leather in such form, viz. a spray, that it (the cement) will coat only the solid portions of the material and not block up the interstices of either the leather or the fabric.

After the composite is thoroughly dried it is pulled off the glass and trimmed. The finished

composite is then cut into strips about 24 inches long which are suitable for hat bands. If desired a pigment finish may be imparted to the leather or both elements of the composite before this final cutting operation.

The composite of leather and fibrous material produced according to my invention in addition to being much less expensive than ordinary leather per se has many decided advantages over leather. The relative low cost of the hat band of my invention is due to the fact that the skivers which can be used as the leather surfacing are very inexpensive in comparison with ordinary leather. In fact as is well known, skivers formerly were discarded as waste material. According to my process, I may employ very weak skins which have hitherto been commercially useless. By means of the reinforcing that I effect I obtain the full benefits of the leather surface and the feel of the leather material without necessitating the use of the customary thicker full leather skins.

However, the thin skiver which of itself could not be used for any useful purpose, when combined with the fibrous material or fabric according to my present invention has sufficient strength and the requisite qualities to be used as a hat band. It is especially noteworthy that the manner of lamination which I have provided hereinbefore makes possible the formation of a strong and yet air pervious reinforced leather.

The hat band of my invention has certain decided advantages over the ordinary leather hat band. First, it holds its shape better inasmuch as the fibrous material to which the leather is securely joined prevents the malformation or distortion of the leather layer. This is an important feature in a hat band. Second, the composite hat band of my invention is more absorbent than the ordinary full leather hat band because the fibrous material which is composited to the leather absorbs perspiration more readily. This again is an important feature inasmuch as it is one of the primary functions of a hat band to prevent perspiration from striking through to the exterior felt of a hat. Thirdly, the hat band is much more uniform in stretch properties than the full leather hat band of the prior art. This is because a full leather hat band is not uniform since it has varying sections of non-uniform texture and stretch. Fourthly, the hat band of my invention can be made in uniform thicknesses. This is obviously desirable in large scale production inasmuch as apparatus for handling hat bands must be carefully adjusted. Plain leather of itself, of course, has varying thicknesses in different sections.

The composite of my invention in addition to being useful for hat bands, as pointed out hereinabove has a special utility in the manufacture of slippers, shoes, gloves, coats, wearing apparel and other fields where reinforced leather can be substituted for a full leather and where air pervious properties are of paramount importance.

Up to this point there has been discussed a novel hat band and the method of manufacturing it. I shall now describe a novel tanning process of my invention which has general application in leather tanning and the specific method of treating leather to obtain the very desirable properties of fine grain texture and superior appearance and any desired flexibility ranging from very soft to rigid. The specific methods and controls, especially the pH controls,

are of great importance and novel results are obtained thereby.

I have also devised a novel method of combining leather with suitable fibrous materials. This combining operation has been described hereinbefore with specific reference to the making of reinforced hat bands. That description is applicable to the manufacturing of composite or reinforced leather for many diverse purposes. In my application Serial No. 72,123, filed April 1, 1936, which has matured into Patent No. 2,132,399, of which this is a continuation in-part, I described generally a method of joining leather to fibrous backing. I shall describe herein certain specific steps which make possible the joining of backing to leather to produce a smooth strong reinforced leather with superior qualities with respect to 'feel' and appearance. The property of "feel" is important inasmuch as leather that has been reinforced by prior methods is thereby stiffened and lacks the softness and flexibility so desirable and necessary in leather.

The method of backing of my invention is of major commercial importance in that it makes possible the utilization of large amounts of skins hitherto without real commercial value. Thus in the field of kid skins, when a large tannery receives a thousand kid skins in the rough, of these thousand skins, after defleshing and dehauling and the usual treatments, 600 of the skins are satisfactory, 200 are too heavy for most purposes and 200 are so light or thin that they cannot be utilized except for linings, etc. These 200 light skins, for example, cannot be used for the manufacture of shoes, etc. as are the satisfactory 600. This has been a very costly circumstance in the leather trade and it is especially irksome because the 200 skins which are too light to be used are actually the finest skins in appearance of the entire lot of 1,000. This is because these very light skins come from the younger and more delicate animals and thus have a finer grain texture and superior appearance. Naturally the appearance and grain of the leather plays a very important part in its value and utility.

It has been impossible to eliminate the waste of these unsatisfactory skins in the past since when the skins are in the rough, their final weight and appearance after treatment cannot be accurately estimated. It has, therefore, been the custom of tanners to dispose of these unsatisfactory very light skins at a low price for uses where strength and stretch are unnecessary, as for linings, pleatings, etc.

In addition to these skins, mentioned above, there are a large number of other light weight skins on the market available at low cost and there are also available skivers which are the splittings from skins of medium or heavy weight. These skivers have insufficient strength to be used by themselves. Skivers are often top grain leather and have a fine appearance but have little value because of their lack of strength.

My novel combining process which has been described generally in my prior application, and specifically herein, makes possible the reinforcing of these light weight skins. In addition to the kid skins I have mentioned, other light weight skins may be backed, such as, for example, snake or reptile skins, buck skins, such as China buck, doeskins, goat skins, sheep skins, etc. By my combining method these light weight skins which may have insufficient strength in themselves to be used for many purposes such as the manufacture of shoes, handbags, hat bands, wearing

apparel, hats, pouches, etc. are reinforced with a backing so that they have the proper strength, a predetermined stretch, and a desirable thickness to render them valuable and useful for these above enumerated purposes. The composites may or may not be air pervious, as desired, depending upon factors such as the method of application of the binder.

It is a further object of my invention, therefore, 10 to provide a novel process for reinforcing skins by applying a backing thereto.

It is a further object of my invention to provide a novel process of backing light weight skins to obtain a reinforced leather of sufficient 15 strength and having a predetermined stretch.

It is a further object of my invention to provide a novel process of backing skins by taking the skin in a wet state from the tanning operation, smoothing or "slicking" out the skin on a rigid smooth surface to which it adheres, applying a fibrous backing thereto, preferably in the form of a fabric with a suitable binder therebetween, the binder being applied either to the leather, the fabric or both.

It is a further object of my invention to provide a novel tanning process and a preliminary treatment before tanning by means of which new and improved properties are obtained in the leather tanned.

25 I shall now describe specifically my novel tanning process and the preliminary treating process by which I obtain new and unexpected results in tanning. It is to be understood that although this process may be used to obtain the novel hat 30 band of my invention and that this process may also be used for the preparation of leather skins before combining in accordance with the herein-described invention, this presently described tanning and preliminary treatment process has general application in the art of leather tanning and is not intended to be restricted to the combining process set forth on the novel hat band of my invention.

35 In order to obtain a soft stretchy leather with a superior grain and fine finish, I subject the leather to certain treatment before the customary tanning operation.

40 Taking ordinary kid skins, I first test the pH value of the skins and when they are slightly acid, as is usually the case I first neutralize them with alkali, as for example, washing soda. For one hundred pounds of kid skins, I form a bath comprising:

45 Aluminum sulphate ( $Al_2(SO_4)_3$ ) \_\_\_\_ pounds \_\_\_\_ 10  
Water ( $H_2O$ ) \_\_\_\_ gallons \_\_\_\_ 50  
Salt ( $NaCl$ ) \_\_\_\_ pounds \_\_\_\_ 22  
Sodium pyrophosphate \_\_\_\_ do \_\_\_\_ 2 1/2

50 To form this bath I first combine the  $NaCl$  and  $H_2O$ , mixing these two components thoroughly and placing the leather therein. Thereupon, I add the aluminum sulphate (alum) and sodium pyrophosphate in five gallons of water, this charge being delivered to the salt and water bath in four 55 portions, every fifteen minutes. It is to be understood that there is a drum running in the bath to thoroughly contact the skins with the reagents. This drum is now run for one hour whereupon there is added 5 pounds of hypo (sodium hypochlorite) in five gallons of water. This solution is added in two portions, two hours apart. The hypo sets the alum. The entire mix is then run for six hours whereupon skins are taken out and drained overnight. The sodium pyrophosphate 60 above referred to has an unusual action whereby

it facilitates the entry of alum into the leather. This treatment above referred to preserves the leather and makes for a finer grain and straightens the fibre of the leather. It further acts to enhance the appearance of the leather after the tanning.

After the skins have thoroughly drained from this preliminary treatment above described, they are placed in a tank containing 50 gallons of water and 22 pounds of salt, whereupon the pH of this solution is tested. The desired pH is 3.5 and, if it is above that figure, sulphuric acid is added to bring it down. After the proper pH value has been reached, 10% of tanolin (chrome acid) is added. The tanolin is added in four portions over a period of six hours and the skins are run in the drum for one hour more after all the tanolin has been added. Thereupon I test the leather to see whether it will stand a temperature of 212° F. If it does not stand this temperature test, I add bicarbonate of soda to bring up the pH value and run it until it does. The range of this temperature test is from 180° to 212° F. and it can readily be determined when the leather fails to stand the test since it quite clearly shrinks and curls up.

After the leather has been run sufficiently long so that it stands the above-mentioned temperature test, it is taken out and drained for 24 to 48 hours. This acts to set the chrome bath tannage.

Thereafter the leather is placed in a drum with water, and fat liquor is added in sufficient quantities depending on the softness required. After the leather is fat liquored, it is taken out and colored. Alternatively the leather may be colored before the fat liquoring.

The preliminary process of treatment above described and the tanning process produces new and unexpected results and have wide application in the leather industry.

When the leather is to be reinforced with a backing, it is taken, after it has been colored and fat liquored, and while still wet or moist, and slickered or smoothed out onto a smooth rigid surface such as glass, oilcloth or Bakelite. Because the skin is still wet, it adheres very closely to this smooth surface and is firmly held thereon. Thereupon there is sprayed onto the skin a combining liquid such as latex, and a fabric which may or may not have been coated with the combining liquid, is applied thereto. The fabric is laid smoothly on the leather while it is held on the smooth rigid surface and the composite is rolled lightly by rolling pressure produced as for example by a rolling pin. As has been indicated the combining liquid is preferably latex, although certain other rubber cements or suitable flexible cements may be employed. The combining liquid is preferably applied by spraying since spraying produces an air pervious composite and also the composite with the best "feel," but it is within the spirit of this invention to apply the combining liquid in any other manner as by spreading if desired.

After the composite has been dried for twenty hours, it is pulled off the smooth surface and, if desired, the leather is staked on a regular staking machine and finished if desired. The staking machine pulls out the leather and adds to the size and gives the leather a better "feel."

What I believe to be of greatest importance in my combining process is the fact that I take the leather and slicker or smooth it out onto a smooth surface, preferably while the leather is still wet or damp from the previous operations.

Although I particularly stated that the leather is preferably taken while still wet from the prior operations, it is within the scope of my invention to take completely finished leather and re-wet the leather and smooth it out over a smooth surface to combine it with a backing material.

Further although I have set forth that the backing material may be fibrous material in the form of a fabric, the fibrous material can also be in the form of separated fibres and applied by spreading. Similarly, other backing materials of many different kinds can be employed.

There is a further problem in the manufacture of reinforced leather that has long been a source of great difficulty. This problem is that of piping, which, in effect, means the wrinkling on the face of the reinforced leather when it is bent about itself. The piping is caused by the fact that the reinforced leather is so constructed that the leather occupies a lesser area than the backing when it is in a curved position with the backing outside, than when it is in a flat position. Thus, because it has been customary in the past to employ a non-elastic backing such as a woven fabric cemented to the leather, when the leather was bent or flexed about itself with the backing on the outside, inasmuch as the non-elastic backing would not "give," the leather was forced to constrict in some manner and the constriction was compensated for by the wrinkle or piping effect. This piping effect is extremely undesirable both from the standpoint of its appearance per se and also because it shows up in the finished article by a wrinkle effect. This is illustrated for example in the manufacture of shoes from reinforced leather. When the leather is curved inwardly on the side of the arch of the shoe, the leather surface of the shoe has a wrinkled or piped effect.

I have conceived of a novel combination whereby this piping effect is completely eliminated, and whereby reinforced or backed leather has under all circumstances of curvature the same desirable smooth unwrinkled surface as unbacked leather itself.

I accomplish the elimination of this piping or wrinkled effect by employing as a backing a material that has a "give" or elasticity equal to or greater than the "give" or elasticity of the fleshy part of the leather. Thus the addition of the reinforcement or backing to the leather has no more constricting effect on the surface of the leather than the normal fleshy portion of the leather itself. In addition to employing this backing material with this property of "give" or elasticity, I further employ a binding agent or cement between the leather (that is, the fleshy part of the leather) and the backing that is extremely flexible and elastic. Preferably, I employ as this binding material or cement, a rubber cement such as latex; the latex preferably should not have contained in it any fillers or modifying agents that would interfere with this desirable very elastic property. The binding agent is preferably placed between the fleshy side of the leather and the backing with the smooth face of the leather on the outside.

For the flexible backing material with the desirable "give" above indicated, I preferably employ a knitted material in contrast to the woven material hitherto employed for backing. Woven material notoriously has a very limited stretch or relatively no stretch at all. Knitted material on the other hand, such as I desire to employ, has a

stretch in all directions, its stretch being for all practical purposes unlimited.

To preserve the desirable smooth surface of the leather, I prefer to employ a knitted material which has little or no design, thus presenting a smooth knitted fabric surface to the fleshy part of the leather, hence transmitting no impression through to the face of the leather. Thus, I may employ a plain smooth knitted fabric of any desired weight or thickness, depending on the particular weight of the product desired. This knitted material may be of cotton, wool, or any suitable material.

Although I have set forth here that I prefer to employ a knitted fabric as a reinforcing for the leather, it is conceivable that a woven material such as lastex or a woven material by a newly devised weave, could be employed, but it is essential that such material have a "give" or stretch that is equal to or greater than the fleshy part of the leather when the leather is curved. As far as I know there is no woven cloth at present that has sufficient stretch to accomplish my purpose, except woven lastex. Thus, for all practical purposes, I may employ a knitted fabric backing.

As a specific example of the method of making this novel non-piping reinforced leather I may take a skin after the dyeing and tanning operations and apply to the fleshy side of the leather the latex or suitable flexible cement by means of spraying. After the latex binder has been deposited on the leather I may apply the knitted fabric on to the binder coated leather. The knitted fabric may itself be given a coating of latex or suitable flexible cement to insure a good binding to the leather. This particular joining of the knitted fabric to the leather may be carried out as hereinbefore indicated in my compositing operations described.

Another method I have found which insures the formation of a composite of leather and backing without piping effects comprises applying the pressure that effects the joining of the fabric to the flexible cement coated leather by means of a multiplicity of prong like extensions. For example, I can employ a brush having relatively stiff bristles which I press down perpendicularly with respect to the fabric positioned on the flexible cement coated leather and thereby effect spaced or spotted adhesion of the reinforcing fabric to the leather.

Preferably the flexible cement is applied in the form of a spray over the leather and this spray may be relatively dense or relatively separated. In other words the cement coating on the leather may be almost continuous, or in fact continuous,

if it is not desired to retain the air pervious qualities of the composite, or, at the other extreme, the cement coating on the leather may be relatively discontinuous and consist in spaced dispersed particles or globules of cement on the leather.

In other words, in order to obtain a bending of the leather about itself without piping or wrinkling, I propose spotting or spot joining of the leather to the reinforcing backing. As I have set forth this spot joining may be accomplished either by dotting one of the members to be joined with spaced spots of adhesive and applying an all over pressure to the composited elements, or by applying a continuous or almost continuous coating of cement to one of the elements and applying a spaced spot pressure to effect the joining of the component parts.

The apparatus for carrying out this spaced pressure joining of the elements comprises preferably a multiplicity of spaced rigid narrow elements of equal length so that an even pressure is distributed throughout the elements to be pressed. Thus, I could employ a plate having distributed thereon a multiplicity of rod-like elements of equal length and apply such plate perpendicularly with respect to the elements to be joined so that the points of the rod-like elements strike the composite to be united.

Although I have set forth that this desirable break can be obtained by spacing the cement particles one from the other or by using a coating of cement and spacing the pressure elements, the latter method has a particular advantage since the cement when in spots has a tendency to show through on the face of the leather. When very thin leather is employed a further advantage results in that the all over uniform coating imparts a uniformity to the final product.

The pressure which I employ to effect the joining when employing the multiplicity of pressure elements ranges from about twenty-five to one hundred and twenty-five pounds per square foot, the exact amount of pressure being determined for the thickness of the elements to be joined and for the use of the final product. The pressure is also determined by the character of the cement.

I claim:

50 A hat band comprising a layer of leather and a knitted fabric united by a layer of cement, said fabric having a greater elasticity than leather, said cement consisting of a latex free fillers to form spaced particles permitting passage of air therethrough.

55

HIMEN COOPER.